

Patented Mar. 4, 1924.

1,485,635

# UNITED STATES PATENT OFFICE.

JOHN MURDOCH SKELLEY, OF LONDON, ENGLAND, ASSIGNOR TO THE CONTINUOUS REACTION COMPANY, LIMITED, OF LONDON, ENGLAND.

## MANUFACTURE OF FERROUS ALLOYS AND OF WEATHERPROOF ARTICLES THEREFROM.

No Drawing.

Application filed June 11, 1923. Serial No. 644,751.

To all whom it may concern:

Be it known that I, JOHN MURDOCH SKELLEY, a subject of the King of Great Britain, residing at 155 Church Road, Battersea, London, England, have invented new and useful Improvements in the Manufacture of Ferrous Alloys and of Weatherproof Articles Therefrom, of which the following is a specification.

- 10 This invention relates to the manufacture of certain ferrous alloys and to the production from such alloys of manufactured articles the use of which involves their exposure to alternate wetting and drying, to 55 damp and varying atmospheric conditions, or to like influences which cause the rusting of articles made of ordinary iron or steel.
- 15 As is well known, polished hardened articles, such as cutlery, of the kind commonly called "stainless", are manufactured from iron-chromium alloys containing about 12 to 15 per cent of chromium and small percentages of carbon, silicon and other constituents.
- 20 In my experience such alloys, although serving for the production of articles which are sufficiently untarnishable under the conditions of domestic use, are of somewhat limited applicability. They cannot be successfully used for the manufacture of unpolished, weatherproof articles, such as implements, fittings, plates, castings, and the like, which have to withstand for long periods 60 exposure to alternate wetting and drying, to 65 damp and varying atmospheric conditions, or to like influences. Moreover, it is necessary both to harden by heat-treatment and to impart a polished surface to articles of that composition in order to render them 70 reasonably untarnishable under the conditions of use for which they are intended. So far as I am aware, no article of such alloys has hitherto been made which, when exposed in a clean but unpolished condition, (for example, after drilling, machining, rough buffing or grinding) to the action 75 of rain and sunshine would not become 80 rusted in the course of a few days.

This invention relates to the manufacture 85 of the iron-chromium alloys hereinafter described and the production from these alloys of manufactured articles, hereinafter called for brevity "weatherproof articles" the use of which involves their exposure to

alternate wetting and drying, to damp and varying atmospheric conditions, or to like influences, and which in a polished or unpolished condition, and whether hardened or not, are capable of withstanding such exposure for prolonged periods without rusting. Examples of such articles are plates, rails, girders, cast objects, automobile parts, utensils, implements and tools for out-door use; ships' fittings; bathroom fittings; burnished fenders; cooking stoves and the like 65 which are liable to have liquid spilt on them.

It is known that iron and chromium can be alloyed with one another in widely different, and probably in all, proportions. It is also known that the alloys rich in chromium are comparatively resistant to the action of acids, but are of little practical interest for the production of manufactured articles owing to their high cost, the difficulty of working them, and their defective 70 physical and mechanical properties. We have discovered, however, that a ferrous alloy containing from 12 to 24 per cent of chromium, from 0.4 to 3 per cent of molybdenum, from 0.05 to 0.85 per cent of carbon 75 and from 0.1 to 1.3 per cent of silicon (the higher the percentage of carbon, the higher the percentage of chromium) can be readily cast or worked and that articles manufactured of it are highly resistant to rusting 80 when used in the rain or otherwise exposed to damp and varying atmospheric influences. I have also found that, the usual minor constituents of commercial steels have 85 little or no prejudicial effect upon the 90 weatherproof properties of articles made of the alloy. It is not necessary either to harden or to polish such articles in order to render them weatherproof, although they may be so treated if desired. When polished 95 they possess the advantageous property that if accidentally scratched or roughened they remain weatherproof.

The invention consists in the manufacture of ferrous alloys containing from 12 to 100 24 per cent of chromium, from 0.4 to 3 per cent of molybdenum, from 0.5 to 0.85 per cent of carbon and from 0.1 to 1.3 per cent of silicon (the higher the percentage of carbon, the higher the percentage of chromium), with or without the usual minor constituents of commercial steels, and in the manufacture of weatherproof articles from 105

the said alloys. Preferably the percentage of carbon in the alloy does not exceed a certain maximum, which depends upon the percentages of chromium and molybdenum 5 present, the rule for determining the preferred composition (herein termed "the rule of maximum carbon percentage") being as follows:—

With 0.4 to 0.5% Mo the maximum 10 percentage of C corresponding to a given percentage Cr should be as stated in the following table (from which intermediate percentages can be deduced):—

| 15 | Alloy containing 0.4-0.5% Mo. |      |
|----|-------------------------------|------|
|    | Cr%                           | C%   |
|    | 12                            | 0.1  |
|    | 14                            | 0.3  |
|    | 16                            | 0.4  |
| 20 | 18                            | 0.55 |
|    | 20                            | 0.65 |
|    | 22                            | 0.75 |
|    | 24                            | 0.85 |

while 0.05% more C is allowable for each 25 additional 0.5% Mo provided always that the percentage of carbon is not more than 0.85; thus an alloy containing 1.5% Mo and 16% Cr should not contain more than 0.5% of C.

30 In carrying the invention into effect the alloy is produced by any convenient method, for example, by melting steel, chromium or ferrochromium and molybdenum or ferromolybdenum in the requisite proportions together in an electric furnace, care being taken to avoid as far as possible any inclusion of chromium oxide, which might otherwise injure the weather-resisting properties of the alloy. Weatherproof articles 35 are then made of the alloy by the following usual methods. If wrought articles are to be produced, the molten metal is cast into ingots and afterwards hammered, rolled or otherwise worked and treated according to 40 known methods, care being taken at all stages to avoid working oxide into the metal, as the presence of particles of oxide on the surface tends to set up rusting. It is not necessary, in order to render the article rust- 45 less, to finish the manufacture by polishing the surface; a simple cleaning by grinding, buffing or the like is sufficient. If the 50

object in view is to produce castings, the molten metal is cast in moulds in the usual way and the dark, oxidized skin may afterwards, if desired, be left on the casting without undue risk of rusting occurring. 55

#### Example 1.

An alloy containing 12.7 per cent of chromium, 1.53 per cent of molybdenum, 0.2 per cent of carbon and 0.3 per cent of silicon is prepared by melting steel along with the required proportions of ferrochromium and ferromolybdenum in an electric furnace. 60

Weatherproof drums are manufactured from the alloy by casting it into an ingot and then hammering and rolling into sheets, which are cleaned by buffing and formed into drums in the usual manner. The alloy 70

can be readily cut and drilled.

Plates made of this alloy, either polished or unpolished and drilled partly through at various points to offer shallow depressions in which rainwater might lodge, have been 75 openly exposed during some weeks of rainy weather and have not rusted.

#### Example 2.

An alloy containing 17.46 per cent of chromium, 0.47 per cent of carbon, 1.2 per cent of silicon and 1.1 per cent of molybdenum is prepared as in Example 1.

Range-finder parts to be used in an exposed situation are manufactured from the 85 alloy by casting it into ingots and working it by usual methods into the desired articles.

What I claim is:—

1. A ferrous alloy containing from 12.90 to 24 per cent of chromium, from 0.4 to 3 per cent of molybdenum, from 0.05 to 0.85 per cent of carbon and from 0.1 to 1.3 per cent of silicon.

2. Weatherproof articles manufactured 95 from a ferrous alloy containing from 12 to 24 per cent of chromium, from 0.4 to 3 per cent of molybdenum, from 0.05 to 0.85 per cent of carbon and from 0.1 to 1.3 per cent of silicon.

In testimony that I claim the foregoing as my invention I have signed my name this 28th day of May, 1923.

JOHN MURDOCH SKELLEY.